

# UNITED STATES PATENT OFFICE.

WILLIAM F. OESTERLE, JR., CLIFFORD A. BEALE, AND JOSEPH MCFETRIDGE, OF VANDERGRIFT, PENNSYLVANIA, ASSIGNEES TO AMERICAN SHEET AND TIN PLATE COMPANY, OF PITTSBURGH, PENNSYLVANIA, A CORPORATION OF NEW JERSEY.

## PROCESS OF UTILIZING WASTE FERROUS LIQUORS.

1,108,387.

Specification of Letters Patent.

Patented Aug. 25, 1914.

No Drawing.

Application filed October 10, 1913. Serial No. 794,413.

To all whom it may concern:

Be it known that we, WILLIAM F. OESTERLE, JR., CLIFFORD A. BEALE, and JOSEPH MCFETRIDGE, citizens of the United States, residing at Vandergrift, county of Westmoreland, and State of Pennsylvania, have invented certain new and useful Improvements in Processes for Utilizing Waste Ferrous Liquors, of which the following is a specification.

This invention relates to a process of treating spent pickle liquors for the purpose of regenerating the liquors, and utilizing the treated liquors for pickling steel or iron.

The process of pickling consists in removing scale, oxids and the like, from the surface of metallic articles, by subjecting the articles to the action of an acid bath, capable of removing the surface defects, and for the purpose of improving the surface appearance or to prepare the articles for subsequent treatment, such as tin plating or galvanizing. The usual practice is to start the operation with a bath containing from 3 to 5 per cent. of a free acid, such as sulfuric or hydrochloric acid. Steel or iron articles are submerged in the bath, and as the acid is neutralized, fresh acid is periodically added. The specific gravity of the liquor increases with each addition of acid and batch of iron treated, and when a strength of from 28 to 30 degrees Baumé is reached the further addition of acid is stopped, and as far as practical the acid is neutralized. When sulfuric acid is used (as is usually the case) this concentrated bath consists principally of ferrous sulfate and a varying per cent. of free acid, and as a medium for pickling steel or iron has no further value and is known to the trade as spent pickle liquor.

It is the object of our invention to recover a portion of the iron in this liquor as rouge or pigment and to convert the remaining amount of ferrous sulfate into ferric and basic ferric sulfate, which we use for pickling steel or iron. It will be evident that in this way all the iron and all the acid value of the liquor are utilized.

By our method of utilizing spent pickle liquors, when the process of pickling is once started with sufficient acid to pickle a given quantity of steel or iron, no further acid is necessary, except what is required to com-

pensate for the mechanical loss in operation. The iron that is combined as ferrous sulfate is used in our process as a means of conveying oxygen, and by a series of steps of oxidation and reduction, the acid is used over and over for pickling steel or iron, although the acid is not isolated as commercial acid, but is mixed with ferric sulfate, which we find has not only a beneficial effect in overcoming defects peculiar to the acid pickling process, but accelerates pickling. The iron removed from the steel or iron during the pickling process is recovered during the regenerating process as ferric oxid, and the quantity of oxid of iron removed is equivalent to the dissolving power of the regenerated liquors.

According to prior methods of utilizing spent pickle liquors, the free acid was neutralized with scrap iron and the liquors concentrated to the crystallizing point, and commercial copperas produced. The commercial copperas was decomposed by heat to form ferric oxid and sulfuric anhydrid was liberated. By other methods, the spent pickle liquors were concentrated to the crystallizing point, and by continuing the evaporation, ferrous liquor salts were obtained. These salts were decomposed by heat to form oxid of iron and sulfuric anhydrid the latter being used in making commercial sulfuric acid. When ferrous sulfate is decomposed into ferric oxid and sulfuric anhydrid the end reaction follows:



Before complete decomposition takes place, a series of intermediate reactions take place as follows: When the temperature is very low, basic ferric sulfate is formed by the reaction



on further heating, the basic ferric sulfate decomposes, forming ferric oxid and ferric sulfate and sulfuric anhydrid is set free, the reaction being



By increasing the temperature, the ferric sulfate decomposes forming ferric oxid and sulfuric anhydrid as follows:



In our process we furnace the ferrous sulfate or ferrous liquor salts, at a temperature below dull red heat, with admission of air and constant stirring of the mass, so that oxidation rapidly takes place, and basic ferric sulfate  $Fe_2O(SO_4)_2$  is formed. By discontinuing the heat at this point or removing the charge, we can retain in the furnace product all the acid value originally contained in the ferrous salts. By digesting the basic ferric sulfate in water, we regenerate sulfuric acid for pickling iron or steel, according to the following reaction:



By decantation and filtration, we remove the ferric oxide as rouge or pigment, and use the filtrate to pickle steel or iron according to the following reaction:



The foregoing is the end reaction when all the ferric sulfate has been reduced to ferrous sulfate and the free acid neutralized. The ferric sulfate which is present prevents the absorption of hydrogen by the iron or steel which is being pickled and also prevents the action of galvanic couples ordinarily caused by the action of the various constituents of iron or steel; for example, it is well known that under ordinary circumstances there is a difference in potential between the pearlite and ferrite of steel which causes the formation of a galvanic couple with consequent electrolytic action. By reason of the results which have just been described, the ferric sulfate acts as a depolarizer and the hydrogen which would under ordinary circumstances be absorbed by the iron or steel is used to reduce the ferric to ferrous sulfate. This depolarizing effect continues until all the ferric sulfate has been reduced to ferrous sulfate. When the pickling operation is continued after all the ferric sulfate has been reduced, we no longer have the depolarizing effect, but the free sulfuric acid acts directly on the steel, producing ferrous sulfate.

When the ferric sulfate has been in part reduced, we prefer to replenish the bath with fresh ferric sulfate (mixed with ferrous sulfate), or with basic ferric sulfate, these salts being produced by the process above described. In the presence of water the basic ferric sulfate breaks up into ferric oxide, ferric sulfate and sulfuric acid. In this way we have the depolarizing effect of the ferric sulfate throughout the entire pickling process, and when the specific gravity of the liquor reaches 30 to 35 degrees Baumé the liquor is drawn off and treated by our above described process.

It is well known that in the regular acid pickling process certain effects are produced

that cause permanent defects in the steel or iron treated. It is also known that galvanic couples are formed simultaneously with the immersion of the steel or iron articles in the acid bath, the electrolytic hydrogen having a tendency to produce sponge at the cathode of the couple, and by absorption of hydrogen, the steel or iron articles are affected in a manner that causes defects in the subsequent treatment of the steel, such as tin plating and galvanizing. By using our process the cause of these defects can be overcome and the defects prevented by accomplishing the pickling in presence of depolarizing salts, such as ferric sulfate or ferric chlorid. Moreover, the presence of ferric salts will produce a uniform crystalline surface on the articles treated.

Having thus described our invention in general terms, we will now describe the various steps in detail:

1st. Waste ferrous sulfate liquors are heated and treated with fine oxid of iron in quantities equivalent to the free acid present, for the purpose of neutralizing the free acid and forming ferric sulfate. The treatment with ferric oxid can be accomplished in any suitable container.

2nd. The liquors are concentrated in any of the well known apparatus for concentrating corrosive liquors, and evaporation of water continued to point of saturation. When the liquor has reached the point of saturation, the temperature and specific gravity of the liquor are such that the free acid dissolves the oxid of iron added in the first step of the process to form ferric sulfate. By continuing the evaporation, ferric sulfate and ferrous sulfate are salted out.

3rd. The mixture of ferric sulfate and ferrous sulfate as produced in the second step of the process is furnace in any suitable furnace at a temperature below dull red heat, with admission of air and constant stirring of the salt, oxidizing the ferrous sulfate into basic ferric sulfate according to the reaction



The ferric salt contained in the mixture being treated remains unchanged at the temperature stated, so that the product of this third step of the process is a mixture of ferric sulfate and basic ferric sulfate.

4th. The product of the third step of the process is digested in water in any suitable apparatus, the ferric sulfate dissolving and the basic ferric sulfate combining with water to form ferric oxide, ferric sulfate and sulfuric acid according to the reaction



5th. The insoluble ferric oxide produced in the fourth step of the process is removed

from the solution by decantation and filtration by any of the well known apparatus used for that purpose, and the ferric oxide is washed to free it from soluble iron salts.

5 The ferric oxide is used to produce pigment.

6th. The filtrate of the fifth step, consisting of a mixture of ferric sulfate and free acid, is utilized for pickling steel or iron, which can be accomplished in any suitable 10 apparatus. The strength of the liquor can vary to suit the requirements of the articles being treated. We find that a solution containing from 2 to 5 per cent. free acid is well adapted to ordinary work. The pickling can be accelerated by raising the temperature; the temperature we have found most suited for usual work is from 130 to 150 degrees Fahrenheit. To this bath we add steel or iron articles, which are rapidly 20 pickled according to the reaction



The hydrogen set free reduces the ferric sulfate to ferrous sulfate, according to the 25 reaction



The bath is replenished from time to time with ferric sulfate, which may be a mixture 30 of ferric sulfate and ferrous sulfate as produced in the second step of the process, or by the mixture of ferric sulfate and free acid as produced in the fifth step. When the strength of the liquor has increased to 30 to 35 degrees Baumé, the addition of ferric sulfate is stopped, and the pickling operation continued until ferric salts are reduced to ferrous salts.

7th. When it is desirable to utilize the 40 free acid contained in the spent liquor from the sixth step of the process, the pickling operation may continue until the free acid is neutralized by the reaction



45 It will be apparent to those skilled in the art that considerable change could be made in the details of the process which we have described without departing from the spirit 50 or scope of our invention.

What we claim is:

1. The process of utilizing spent ferrous liquor, which consists in oxidizing the ferrous to ferric salts, and adding said ferric 55 salts to an acid cleaning solution, whereby polarization is prevented in the presence of a metal to be cleaned, substantially as described.

2. The process of utilizing spent ferrous 60 liquor, which consists in neutralizing the free acid in said liquor, oxidizing the ferrous

to ferric salts, and adding said ferric salts to an acid cleaning solution, whereby polarization is prevented in the presence of a metal to be cleaned, substantially as described. 65

3. The process of utilizing spent ferrous liquor, which consists in treating the liquor with ferric oxide to neutralize the free acid with the formation of a ferric salt, oxidizing the ferrous to ferric salts, and adding said 70 ferric salts to an acid cleaning solution, whereby polarization is prevented in the presence of a metal to be cleaned, substantially as described.

4. The process of utilizing spent ferrous liquor, which consists in neutralizing the free acid of said liquor, furnacing to oxidize the ferrous to ferric salts, digesting with water to dissolve the soluble salts, and adding said solution to an acid cleaning solution, whereby in the presence of a metal to be cleaned polarization is prevented, substantially as described. 75

5. The process of utilizing spent ferrous liquor, which consists in neutralizing the free acid of said liquor, furnacing to oxidize the ferrous to ferric salts, digesting with water to dissolve the soluble salts, filtering to separate the soluble from the insoluble salts, and adding the filtrate to an acid cleaning solution, whereby in the presence of a metal to be cleaned the ferric salts are reduced to ferrous salts and polarization is 80 prevented, substantially as described. 85

6. The process of utilizing spent ferrous sulfate liquor, which consists in neutralizing the free acid in said liquor, evaporating said liquor, whereby the dissolved salts are separated out, oxidizing said salts to form ferric sulfate and adding said ferric sulfate to an acid sulfate cleaning liquor, whereby in the presence of iron said ferric sulfate is reduced to ferrous sulfate and polarization is 90 prevented, substantially as described. 95

7. The process of utilizing spent ferrous sulfate liquor, which consists in neutralizing the free acid in said liquor, evaporating said liquor, whereby the dissolved salts are separated out, oxidizing said salts to form ferric sulfate, treating said salts with water, filtering to separate oxid of iron from the soluble ferric sulfate, and adding said filtrate to an acid sulfate cleaning liquor, whereby in the presence of iron said ferric sulfate is reduced to ferrous sulfate and polarization is 100 prevented, substantially as described. 110

WILLIAM F. OESTERLE, JR.

CLIFFORD A. BEALE.

JOSEPH McFETRIDGE.

Witnesses:

SAMUEL K. HUNGER,  
JOHN W. HUNGER.